

## UNITED STATES PATENT OFFICE.

VAN CORTRIGHT MEKEEL, OF HIGH BRIDGE, NEW JERSEY, ASSIGNOR TO TAYLOR-WHARTON IRON AND STEEL COMPANY, OF HIGH BRIDGE, NEW JERSEY, A CORPORATION OF NEW JERSEY.

## METHOD OF TREATING MANGANESE STEEL.

No Drawing.

Application filed February 27, 1928. Serial No. 91,267.

My invention relates to the treatment of iron and steel alloys and more particularly manganese steel.

Objects of the invention are to provide for increased strength, and especially greater resistance to abrasive wear, of manganese steel shapes or articles, whether formed by casting or working or both, without impairing the toughness and ductility of the metal.

10 The nature of my invention consists in sealing manganese steel castings or forgings in the presence of case hardening or cementation material, effecting the case hardening during the heating operation in heat treatment, and quenching the case hardening product under conditions conducive to minimum exposure to the air. By varying the material as to its components and their relative proportions, and by regulating the time the 15 charge is held at heat, the depth and nature of the case hardening can readily be controlled.

According to my invention, I provide for case carbonizing, case boronizing, or both, by 20 subjecting the casting or forging to the action of carbonizing or boronizing materials, or a mixture thereof, while sealed against the atmosphere, during the heating stages in heat treatment. Examples of materials appropriate for the purpose are barium carbonate ( $BaCO_3$ ) and charcoal or coke; boric 25 oxide or boric alloy, in a finely divided state, with suitable reducing agents. In practice, the casting or forging and the charge are 30 sealed in a container, or in a covering, the nature of which will depend upon the size and shape of the article and whether it is being treated singly or in quantities, but which, by preference, will be adapted to admit of 35 quenching of the article or articles with little or no exposure to the air. An example is 40 disclosed in my co-pending application, Ser. No. 91,113.

My invention applies to high per cent manganese steel or what is known as commercial manganese steel, that is to say, steel having a manganese content ranging from five to twenty per cent and preferably eleven to fourteen per cent.

In some cases I propose to line the molds 45 with finely divided boric oxid or boric alloy in admixture with various reducing substances and utilize the heat of casting to fuse boron into the surface of high per cent manganese steel.

Having described my invention, I claim:

1. The method of imparting greater strength and wear resistive properties to manganese steel without impairing the toughness and ductility of the metal, which 50 consists in case hardening the shape during the regular heat treatment, and quenching under conditions conducive to minimum exposure to air.

2. The method of imparting greater 55 strength and wear resistive properties to manganese steel without impairing its toughness and ductility, which consists in packing the shape with cementing material in a container and, while so sealed against 60 exposure, heat treating in the regular way, and then quenching.

3. The method of imparting greater 65 strength and wear resistive properties to manganese steel without impairing its 70 toughness and ductility, which consists in sealing the shape in the presence of finely divided boric oxid and a reducing agent, and, while so sealed, heating it in stages in 75 the regular order of heat treatment, and then 80 quenching.

In testimony whereof I affix my signature.

VAN CORTRIGHT MEKEEL.